

## UNITED STATES PATENT OFFICE.

ARTHUR LEE BROWNE, OF BALTIMORE, MARYLAND, ASSIGNOR TO THE AMERICAN HAMMERED PISTON RING COMPANY, OF BALTIMORE, MARYLAND, A CORPORATION OF MARYLAND.

## VALVE-GRINDING COMPOUND.

No Drawing.

Application filed August 29, 1927. Serial No. 216,346.

Until quite recently grinding, or lapping compounds, and more particularly those for grinding the valves of automobiles, have consisted of a mixture of abrasives such as 5  
5 emery, carborundum, or corundum, and a heavy grease. There are, however, several objections to a grinding compound in which a grease is used as the binder.

(a) Owing to the fact that the grease acts 10 as a lubricant during the grinding operation, the abrasive grains do not break down, but continue to cut and imbed themselves in the articles being ground; and therefore, it is necessary to finish grind, or lap, with a finer 15 grade of abrasive. To obtain the proper finish on the surface being ground, when using a grease-mixed compound, it is necessary, therefore, first to use a coarse grade of abrasive for the cutting operation, and to 20 finish with a fine grade to obtain a polish.

(b) It is difficult to clean the surfaces that have been lapped or ground, with a grease-mixed compound, and particularly is this true when grinding the valve seats in automobiles. Inability to clean the valve seats 25 perfectly in an automobile after grinding, naturally causes very serious results, as the emery, carborundum, or other abrasive used, soon causes wear, and should this abrasive 30 get down into the cylinders it would cause an untold amount of trouble due to cutting action upon the piston rings, piston and cylinder. Furthermore, a grease-mixed compound is greatly affected by climatic changes, 35 becoming quite fluid in excessively hot weather, and extremely stiff in very cold weather.

In view of the above disadvantages, the so-called water-mixed grinding compound 40 has come into use in recent years, and particularly for grinding the valves of automobiles. The water-mixed compound has the advantage of allowing the use of a well graded mixture of abrasive or carborundum 45 grit, which cuts quite rapidly at first, but owing to the friction produced by grinding, the particles soon break down into smaller particles, which with the continued grinding action produce a highly polished surface. 50 Consequently, with water-mixed compound it is not necessary to use two grades of abrasive, but one medium grade or well propor-

tioned mixture of abrasive or carborundum grit will serve both for the roughing and finishing out, and/or final polish.

There are certain disadvantages to the water-mixed compounds, however, which may be stated as follows: First, it has a tendency to rust the surface upon which it is used, necessitating very careful cleaning 55 of the article after grinding, and a thorough oiling of same to prevent the subsequent formation of rust. It has been noticed that with the majority of valve grinding compounds now on the market, the rusting action 60 is very rapid, and frequently the article being ground is rusted before the valve grinding compound is thoroughly removed, the article dried, and the final coating of oil applied. Consequently, a grinding compound 65 that will prevent the rapid formation of rust would be a decided advantage to the industry. 70

Secondly, the water-mixed compounds have a tendency to dry out very rapidly, and 75 it is necessary to keep the container holding the grinding compound closed at all times, in order to prevent the grinding compound from drying out to such an extent that it is useless unless it is again well mixed with 80 the addition of water, and even then, it is seldom as good as was the original mixture. The rapid drying action of the grinding compound necessitates frequent application 85 of water to the article while grinding, and this is objectionable to the users.

Furthermore, with the water-mixed compound, there is, of course, the possibility of such compound freezing in very cold climates. In some of these water-mixed compounds substances have been added to the compound to prevent freezing, and also to lessen the tendency of these compounds to dry, but it is well known in the trade that none of these mixtures have proved entirely 90 satisfactory and all of the compounds now on the market have a tendency to dry out 95 very rapidly, which is perhaps, their most serious disadvantage.

In the valve grinding compound to be now 100 described and forming the present invention the chief difficulties with the water-mixed compounds heretofore on the market, and as above set forth, are overcome, since the

compound will not cause the formation of rust but will actually prevent rust, and furthermore, will not dry out or be affected by climatic conditions.

5 In the grinding compound of this invention, there is used a medium fine grade of abrasive, such as carborundum grade 180. This grade consists mainly of grit that will pass 180 mesh sieve, but it also contains a 10 small amount of coarser particles as well as a small amount of very fine particles. It has been found that by the use of this grade of abrasive a grinding compound can be produced which will cut quite rapidly at first 15 but which eventually breaks down into a finer abrasive powder, during the grinding operation, and produces a high polish.

The abrasive is mixed with a binder or vehicle consisting mainly of glycerine and 20 soap. The glycerine is first heated to a moderate heat for example to 200° F., say by placing the glycerine in a steam bath, and to the warm glycerine a certain amount of soap is added. The soap can be common 25 laundry soap, yellow or white in color, and in the solid state as found on the market, or dried, if desired. Upon mixing, this produces a jellylike substance which acts as an ideal binder for the abrasive material. To 30 prevent this binder from becoming too thin under the influence of heat a small amount of oleic or other fatty acid is added, and after mixing the whole there is added a dilute solution of silicate of soda (about 1 35 part of silicate of soda solution (water-glass) and 4 parts water). While oleic acid is here mentioned, other fatty acids such as palmitic or stearic can be used, in fact any fatty acid which will combine with an alkali to form a soap.

40 This produces a soft jellylike binder unaffected by climatic conditions, and furthermore the composition will not dry out or cause the formation of rust. To this binder the abrasive is added. It will be understood 45 that while carborundum will be particularly referred to herein, various other solid abrasive substances, as corundum, emery and others, may be employed. When the binder and abrasive are mixed together the binder is preferably heated to a moderate heat (say 50 140° F.), and held at this temperature while the proper proportion of abrasive is added and the whole thoroughly mixed. After 55 cooling the grinding compound is ready for use and can be packed in cans or other suitable containers convenient for handling and marketing.

Without attempting to restrict the invention 60 to any particular theory, it is believed that the oleic or other free fatty acid reacts with the sodium silicate to form a soap and a gel of silicic acid or "silica gel". The silicic acid so formed is thoroughly and intimately incorporated with the soap formed

and that originally added, together with the water and glycerine, constitute the base or vehicle of the composition, giving the desired soft jellylike consistency, and aiding in holding the water in the composition during use.

It is desired to call attention to the fact that the composition is stable at all ordinary temperatures. It does not freeze in winter, nor does it change its consistency at freezing 75 temperatures, and can be even heated to 180° F., without any separation occurring. Furthermore, the soapy film which is left after wiping or removing the material inhibits rust.

Without restricting the invention thereto, the following examples of compositions falling within the scope of the invention are given, for the purpose of illustration:

|                      | Per cent. |
|----------------------|-----------|
| Carborundum          | 50        |
| Glycerine            | 24        |
| Soap                 | 4         |
| Stearic acid         | 3         |
| 30% silicate of soda | 4         |
| Water                | 15        |

#### Example 1.

|                         | Per cent. |
|-------------------------|-----------|
| Carborundum             | 40        |
| Glycerine               | 30        |
| Soap                    | 5         |
| Oleic acid              | 4 to 6    |
| 30-40% silicate of soda | 3 to 5    |
| Water                   | 16        |

#### Example 2.

A grinding compound composed of the following ingredients, which compound will not be as stiff as the former:

|                         | Per cent. |
|-------------------------|-----------|
| Carborundum             | 40        |
| Glycerine               | 30        |
| Soap                    | 5         |
| Oleic acid              | 4 to 6    |
| 30-40% silicate of soda | 3 to 5    |
| Water                   | 16        |

#### Example 3.

A particularly favorable formula, for making the product, is as follows:

|                                  | Per cent. |
|----------------------------------|-----------|
| Glycerine                        | 30        |
| Soap                             | 5         |
| Oleic acid                       | 6         |
| 40% solution of silicate of soda | 4         |
| Water                            | 15        |
| Carborundum                      | 40        |

I claim:

1. A paste-like abrasive material containing the reaction products of alkali metal silicate and a fatty acid together with soap, water, glycerine and a solid finely divided abrasive material.

2. A paste-like abrasive material containing the reaction products of sodium silicate and a fatty acid together with soap, water, glycerine and a solid finely divided abrasive material.

3. A pasty abrasive material containing a pulverulent abrasive material carried in a vehicle containing silica gel and soap.

4. A pasty abrasive material containing a pulverulent abrasive material carried in a vehicle containing silica gel and soap together with water and a substance capable of preventing rapid drying out of the water.

Glycerine 30%; soap 5%; oleic acid 6%; 40% solution of silicate of soda 4%; water 15%; and carborundum 40%.

10

In testimony whereof I have signed my name to this specification.

5. A pasty abrasive material consisting essentially of the following ingredients:

ARTHUR LEE BROWNE.